

## UNITED STATES PATENT OFFICE

2,231,513

## LIQUID FUEL

Albert L. Stillman, Plainfield, N. J., assignor to  
 Fuel Research Corporation, a corporation of  
 Delaware

No Drawing. Application November 5, 1938,  
 Serial No. 238,973

7 Claims. (Cl. 44—8)

This invention relates to improvements in the production of suspensions of coal in oil and has for its principal object to provide a substantially stable suspension of coal particles in hydrocarbon liquid which will be suitable for combustion in furnaces adapted for the burning of oil fuel and other industrial uses, such as, a carburetant in the carbureting of water gas, a binder for coal briquettes and, in general, for all those purposes where 100% oil is now employed but which may be replaced by the suspension of this invention.

In view of the economy which may be realized by a product of this type because of the relative cheapness of solid fuel, previous attempts have been made to produce a satisfactory fuel of coal and oil and while such prior fuels have been satisfactory as fuels they possessed other disadvantages which offset the economies derived from supplementing the oil by coal. For example, it is a matter of experience that when coal and oil are mixed together as they have been in the past, the coal will in time settle to the bottom of the container. Such segregation of the coal renders the mixture useless for the purpose for which it was intended as it cannot be conveniently pumped and several methods were adopted for the purpose of maintaining the coal in suspension, or in other words, to insure the stability of the mixture. One of these methods was to keep the mix in a state of constant agitation by mechanical means. If the mixture was used as a fuel, especially for marine purposes where the fuel is required to stand long periods of storage without precipitation, the use of mechanical agitators was too expensive and their bulk too cumbersome for ship bunkers or fuel storage stations. Another method that was devised was to add to the coal-oil mixture a stabilizer, usually a coagulant such as casein or starch. The disadvantage of this method however is that the use of a coagulant, forming as it does a "gel" of the mix, causes the viscosity of the mixture to become extremely high thereby making preheating and pumping of the mixture difficult and increasing the expense of dispensing the coal in the carrying medium.

I have found that a satisfactory oil and coal mixture which will remain substantially stable for a long period without the necessity of incorporating a coagulant in the mix or using a mechanical agitator, can be obtained if a certain proportion of the coal particles is made sufficiently small and is sufficiently soluble in the oil to produce the phenomenon known as "Brownian Movement." This movement is an

erratic motion which the mass of certain finely divided solid particles effects when suspended in certain fluid media and which for any particle that is moving continues more or less indefinitely in such media. Chemists are not agreed as to the cause of this movement but it is applicant's belief which is in line with the theory advanced by Arthur F. Taggart, T. C. Taylor and A. F. Knoll in their paper issued as Technical Publication No. 312 by the American Institute of Mining and Metallurgical Engineers, that it is due to a chemical action, a partial ionization of the minute solid particles by the liquid media. As a result of the reaction, it is believed that the non-anchored ions on the surfaces of the particles are gradually replaced by less soluble ions from the liquid media and during this change of the surfaces of the particles from a relatively soluble to a relatively insoluble state which takes place at random over the entire surfaces of the particles, an unbalanced or constantly changing mean pull is exerted on each of the particles thereby inducing the particles to move erratically in the liquid media. The essentials for this movement are believed to be, first, that the particle be of a chemical composition that is, second, capable of being ionized to a sufficient but not too great an extent in the liquid media so as to cause the particles to move erratically in such media and, third, that the particles be sufficiently small to be maintained in suspension by such movement.

Coal is known to have been formed from vegetable matter more or less consolidated by the action of heat and pressure. As a result of the coalification process the originally relatively simple molecules are condensed and polymerized to form a much more complex coal molecule whose chemical composition ranges over wide limits, depending on the nature of the original vegetation, on the conditions in the early stages of its deposition and on the magnitude of the natural forces to which the deposit was later subjected. Investigations of the reactions of coal with simple chemical reagents, however, have tended to prove that the coal molecule contains as an essential element of structure, the six-membered carbon ring characteristic of aromatic compounds (The Chemical: Coal by H. H. Lowry, published by the Coal Research Laboratory, Carnegie Institute of Technology, February, 1934). While all coal molecules may have the same essential chemical structure, I have found that coals of the semi-bituminous type which have a high grindability, namely a grindability about 85 on the

Hardgrove scale, are best suited for the purposes of this invention. Bituminous coals may also be satisfactorily used but they should preferably be first heated to the softening point so that they swell and become porous before subjecting them to the grinding operation. The preheating of such coals should be carried to temperatures approximating 350° F. in order to add 40 to 50 percent grindability to the coal which is then preferably ground by a dry-grinding process.

I have found that good results are obtained by mixing with a coal of the above indicated type a hydrocarbon liquid used as liquid fuel (cracked fuel oil). This type of oil is capable of so partially ionizing small particles of bituminous and semi-bituminous coal as to produce the phenomenon above described. The size of the particles at which such movement begins is about .007 millimeter, that is to say, 7 microns. The movement increases in intensity as the particle size decreases and I prefer for the purposes of the invention to reduce the size of the particles to 5 microns as I have found that best results are obtained within practical limits at that size. By grinding the coal and oil mixture together until at least 30 to 50% of the coal particles have been reduced to at least the size of 7 microns and preferably of 5 microns I have found that the mixture will be in a state of microscopic agitation throughout its bulk and that the agitation of the smaller particles will be sufficient to maintain the larger particles in suspension, permanently, the latter remaining equally distributed in a stable state throughout the mixture.

In order that a better understanding of the invention may be obtained, the following example is given by way of illustration:

coal particles which are of micron size. As a specific test, 100 cu. cm. of the mix is removed from the grinder and the coal extracted with carbon bisulfide. The coal is then screened to determine whether it will all go through a 325 mesh screen. If the coal screens as indicated, a portion of it is placed under a microscope to determine the percent of micron size. I have found that a stable mixture of the coal and oil is formed when at least 30% by weight of the coal has been reduced to at least a size of 7 microns and preferably 5 microns and from a practical viewpoint coal particles small enough to produce the "Brownian Movement" will be present in the mixture in efficient proportion to accomplish the purposes of the invention if the proportion of coal particles in the mixture which have been reduced to less than 10 micron size is at least approximately 50% of the coal. In other words, a coal ground to pass 100% through a 325 mesh and having at least 50% by weight of its particles under 10 microns in size will usually have at least 30% of its particles capable of producing Brownian movement of sufficient intensity to stabilize the larger particles of coal. Best practical results, however, are attained if the proportion of coal particles in the mixture under 10 micron size is approximately from 60 to 65% of the coal. The resulting mixture will have a viscosity which is well within the standards of the United States Government for Bunker C fuel oil and can therefore be used with present equipment. The ignition point of the mixture is approximately 425° F. which makes it desirable for use in low rating furnaces.

While I have referred to Pocahontas and lower Kittanning coal in the foregoing example it will be understood that any satisfactory bituminous

- to 70% by weight of a fuel oil having a chemical composition such that it reacts with the coal particles to cause those particles capable of partaking of Brownian movement to move erratically therein and of from approximately 60 to 30% by weight of coal of the bituminous type which has been subjected to a grinding action in the presence of the oil so that it passes 100% through a sieve of about 325 mesh, a substantial portion of said coal particles being of a size as to render them in and of themselves incapable of remaining in permanent suspension in the oil and at least 30% by weight of the coal particles being less than 7 microns but being greater than 5 microns but being greater than colloidal in size and producing in the oil Brownian movement of sufficient intensity to stabilize the larger particles of coal without the aid of other agents. 5
2. A stable liquid fuel having coal particles equally distributed throughout the fuel and composed of a mixture of approximately from 40 to 60% by weight of a fuel oil having a chemical composition such that it reacts with the coal particles to cause those particles capable of partaking of Brownian movement to move erratically therein and of approximately from 60 to 40% by weight of coal of high grindability, at least 30% by weight of the coal particles being less than 5 microns but being greater than colloidal in size and the balance of the coal particles being greater than 5 microns in size but not substantially greater than 325 mesh, the major portion of the coal particles above 5 microns in size being in and of themselves incapable of remaining in permanent suspension in the oil and the particles of coal under 5 microns in size producing in the oil Brownian movement of sufficient intensity to stabilize the larger particles of coal without the aid of other agents. 10
3. A stable liquid fuel having coal particles equally distributed throughout the fuel and composed of a mixture of approximately from 40 to 70% by weight of a fuel oil having a chemical composition such that it reacts with the coal particles to cause those particles capable of partaking of Brownian movement to move erratically therein and of approximately from 60 to 30% by weight of a coal of the bituminous type having a grindability above 85 on the Hardgrove scale, at least 50% of the coal particles being less than 10 microns but greater than colloidal in size and the balance of the coal particles being greater than 10 microns in size but small enough to pass 100% through a sieve of 325 mesh, the coal particles above 10 microns in size being in and of themselves incapable of remaining in permanent suspension in the oil and the particles of coal under 10 microns in size including an amount of coal particles sufficiently small to produce in the oil Brownian movement of sufficient intensity to stabilize the other particles of coal without the aid of other agents. 15
4. A stable liquid fuel having coal particles equally distributed throughout the fuel and composed of a mixture of approximately from 40 to 60% by weight of Bunker C fuel oil and of approximately from 60 to 40% by weight of a bituminous coal having a high grindability, said coal being pulverized so that it passes 100% through a sieve of 325 mesh, a substantial portion of said coal particles being of a size as to render them in and of themselves incapable of remaining in permanent suspension in the oil, and from 30 to 50% by weight of the coal particles being less than from 5 to 7 microns but greater than colloidal in size and producing in the oil Brownian movement of sufficient intensity to stabilize the larger particles of coal without the aid of other agents. 20
5. The method of manufacturing a stable liquid fuel which comprises mixing a coal of the bituminous type having a high grindability, with a fuel oil having a chemical composition such that it reacts with the coal particles to cause those particles capable of partaking of Brownian movement to move erratically therein, until the percentage of coal particles in the mix is greater than 30% but not substantially greater than 60% by weight of the mix, then subjecting the coal in the presence of the oil to a grinding action and continuing such grinding action until approximately all of the coal particles are less than 325 mesh but include a substantial proportion of particles of a size as to render them of themselves incapable of remaining in permanent suspension in the oil and until at least 30% by weight of such coal particles are less than 7 microns but greater than colloidal in size and are capable of producing in the oil Brownian movement of sufficient intensity to stabilize the larger particles of coal without the aid of added stabilizing agents. 25
6. The method of manufacturing a stable liquid fuel which comprises mixing a fuel oil of the order of Bunker C fuel oil with particles of coal until the percentage of coal particles in the mix is greater than 30% but not greater than 60% by weight of the mix, then subjecting the coal in the presence of the oil to a grinding action and continuing such grinding action until approximately all of the coal particles are less than 325 mesh but include a substantial proportion of particles of a size as to render them of themselves incapable of remaining in permanent suspension in the oil and until at least 30% by weight of the coal particles are less than 7 microns but greater than colloidal in size and are capable of producing in the oil Brownian movement of sufficient intensity to stabilize the particles of coal above 7 microns in size without the aid of added stabilizing agents. 30
7. A stable liquid fuel free from added stabilizing agents and composed of fuel oil of the order of Bunker C fuel oil and coal particles equally distributed throughout the oil, the coal in the fuel constituting approximately from 30 to 60% by weight of the coal-oil mixture and being practically free of particles greater than 325 mesh, a substantial portion of said coal particles being of a size as to render them of themselves incapable of remaining in permanent suspension in the oil and approximately 30% of said coal particles being less than 7 microns in size and producing in the oil Brownian movement of such intensity as to stabilize the larger particles of coal in the oil without the aid of other agents. 35

ALBERT L. STILLMAN.